

# UNITED STATES PATENT OFFICE.

WILLIAM N. BLAKEMAN, JR., OF MOUNT VERNON, NEW YORK.

## MINERAL OIL.

1,385,035.

Specification of Letters Patent.

Patented July 19, 1921.

No Drawing.

Application filed February 9, 1921. Serial No. 443,671.

To all whom it may concern:

Be it known that I, WILLIAM N. BLAKEMAN, Jr., a citizen of the United States, and resident of the city of Mount Vernon, in the county of Westchester and State of New York, have invented a new and useful Improvement in Mineral Oils, which invention is fully set forth in the following specification.

- 10 The invention relates to the mineral hydrocarbons obtained chiefly from the Texas, Gulf, and California oil fields. The oils in this class, or group, of which the "Texas oils" are regarded as the type, are known 15 commercially as "asphaltic base oils", and are recognized chemically as being largely composed of unsaturated hydrocarbons.

In applications Nos. 174255 and 174256, filed June 12, 1917, I have described and 20 claimed the utilization of these Texas oils in the arts—particularly in paint-vehicles—by combining them with fatty oils; and the object of the present invention is so to treat these Texas oils that their combining powers 25 will be very greatly increased when brought into contact with drying, semi-drying and non-drying fatty oils and oxidizable matter. This I accomplish by incorporating with the Texas oil a proportion of tung oil.

30 Either the crude mineral oil or any of its fractions, distillates, or residuals, may be used in carrying out my invention, and hence by the term "Texas oil", "hydrocarbon", or "mineral oil", as used in this specification and in the claims, I intend to include the crude oil and also the fractions, distillates, and residuals. The specific oil which I have employed is that from the Sour Lake district, Texas, preferably the available distillates now on the market varying from .92 to .94 sp. gr. The specific gravity of the crude oil varies from .90 to .92 and that of the residuals from .990 to 1.000.

In demonstration of my invention I select 45 a distillate of a light straw color and of .9340 sp. gr., and mix therewith from 15% to 20% of tung oil. This mixture should be subjected to prolonged contact either in broad sunlight, or at a moderate temperature, or both, or at a higher temperature for a shorter time, until the oils are thoroughly blended. A temperature within 250° Fahr. will be found sufficient for general purposes, although the heat may be raised 55 to incipient decomposition if desired. If the mixture be subjected to a heat of 250°

for a short time, and then allowed to blend for about 48 hours, the mixture, when spread on a plain surface, will not break, run, nor separate, but will exhibit a pellicle or cuticle 60 when placed in broad sunlight for about six hours, under favorable atmospheric conditions.

The Texas oil, treated with tung oil, as above described, will readily unite with all 65 the drying, semi-drying, and non-drying fatty oils, in varying proportions, and drying-oil compositions, of any character desired, may be built up therewith. Such drying-oil compositions, even where made 70 with non-drying fatty oils, may be employed in various plastic compositions, and will constitute a new vehicle for paints, as described in my applications Nos. 174255 and 174256.

75 The percentage of tung oil to be used may be varied in practice to meet varying requirements, and will depend upon the gravity and condition of the Texas oil, the character of the fatty oil with which it is 80 to be mixed, and the purpose for which the composition is to be used. As little as 5% of tung oil in the Texas oil will result in the formation of a delicate pellicle on long exposure to favorable atmospheric conditions; but it may be found desirable, in some cases, in forming the mixture of Texas and tung oils, to use the tung oil in excess; so that, when this mixture is combined with the fatty oil, the ultimate composition will 85 show a sufficient percentage of tung oil—an average of 15% of tung oil in the ultimate composition being a good proportion. As a general rule, the non-drying fatty oils will require a larger percentage of tung oil than 90 the semi-drying and drying oils, the percentage decreasing as the drying quality of the fatty oil increases. Thus cotton oil will require 25 parts of Texas oil carrying from 15 to 18 parts of tung oil; sunflower seed oil 100 will require 25 parts of Texas oil carrying from 10 to 12 parts of tung oil; while soya bean oil will require 20 parts of Texas oil carrying from 8 to 10 parts of tung oil.

The Texas oil may, if desired, be oxidized, 105 or hydrogenated, or both, as described in my applications above referred to and in applications Nos. 443,672 and 443,673, filed herewith. The tung oil will be found sufficiently active in its normal condition, when 110 water free, for ordinary mixtures or compositions, but, if desired to accelerate its

affinity, it may be oxidized, or hydrogenated, or both. The oxidization may be effected by heating it on oxidizers, such as the higher oxids of manganese, in the presence of an oxygen-carrier (such as turpentine spirits) if desired; and the hydrogenation may be effected by subjecting the oil, with heat, to the action of hydrogen, in the presence of catalysts. In so treating the tung oil, however, care should be taken in the regulation of heat, as the tung oil, at temperatures approaching 400° Fahr., has a tendency to gelatinize and pass to a solid state, which renders it insoluble in other oils. A satisfactory accelerating action may be given to the tung oil, without using oxidizers, by merely heating it to a temperature of from 250° to 300° Fahr., until a slight deepening of color and thickening of body are indicated, showing an incipient oxidation, and such thickened oil will exhibit increased activity when mixed with the Texas oil. A mixture of Texas oil and 15 to 20% of this thickened tung oil, when properly blended and spread on a plain

surface, will exhibit a pellicle or cuticle in from 8 to 10 hours if exposed in the dark under unfavorable atmospheric conditions, and in about half that time if exposed to broad sunlight.

30

When the tung oil has been treated in any of the ways above described, and thus rendered more active, a smaller percentage may be used with the Texas oil, if desired.

Having thus fully described my invention, I claim:

1. As a new composition of matter, a mixture of a mineral oil of the Texas oil type, and tung oil.
2. As a new composition of matter, a mixture of mineral oil, of the Texas oil type, and oxidized tung oil.
3. As a new composition of matter, a mixture of a mineral oil, of the Texas oil type, and tung oil oxidized and hydrogenated.

35

40

45

WM. N. BLAKEMAN, Jr.

Witnesses:

FRANCIS P. REILLY,  
PASQUALE JOSEPH STIRO.